

## UNITED STATES PATENT OFFICE

HOWARD M. CYR AND ROBERT K. WARING, OF PALMERTON, PENNSYLVANIA, ASSIGNEES TO THE NEW JERSEY ZINC COMPANY, OF NEW YORK, N. Y., A CORPORATION OF NEW JERSEY

## TREATMENT OF ZINCIFEROUS MATERIALS CONTAINING CADMIUM

No Drawing. Application filed October 15, 1929. Serial No. 399,875.

This invention relates to the treatment of zinciferous materials containing cadmium and perhaps other contaminating metals. The invention aims to provide an improved method of effecting a substantial removal or elimination of cadmium from such zinciferous materials without any appreciable loss of zinc. More particularly, the invention contemplates an improved pyrometallurgical treatment for so reducing the cadmium content of zinciferous materials, without substantial loss of zinc, that high grade zinc products can be produced therefrom by customary methods of smelting. While of more especial technical advantage in removing cadmium, the invention contemplates the removal from zinciferous material of other contaminating metals, particularly lead.

Cadmium and zinc are very similar metallic elements in both chemical and physical properties. Indeed, in the zinc industry and in text books on metallurgy, it is common to think and treat of these two metals as very closely related. In all pyrometallurgical processes of zinc extraction, the cadmium follows the zinc, so that no complete separation of the two metals is possible. Accordingly, the presence of a relatively small percentage of cadmium in a zinc ore, or other zinciferous material, prevents the pyrometallurgical production therefrom of high grade zinc products, such as zinc metal, zinc oxide, zinc dust, etc., substantially free of cadmium. Cadmium and lead are technically the most commonly recognized contaminants of zinc ores and their concentrates. In addition, certain metals, such as tin, antimony, bismuth, etc. are commonly present in zinc ores. Appreciable amounts of these contaminating metals, more especially cadmium and lead, find their way into the product of the zinc recovery operation and thereby contaminate the zinc product obtained therefrom.

In the copending patent application of Lloyd E. Teter, Serial No. 371,058, filed June 14, 1929, there is disclosed and claimed a method of removing cadmium and/or lead from zinciferous material by subjecting the material to a sintering operation by blast-

roasting in the presence of a chloridizing agent and water vapor. While sodium chloride would appear to be the most available and economical chloridizing agent in the practice of that method, we have discovered, in the course of a thorough and careful practical investigation of the method, that sodium chloride and similar chlorides of elements capable of forming strong bases, so react in the course of the sintering operation as to render a large proportion of the chlorine present unavailable for its contemplated action in chloridizing cadmium and/or lead. For this reason, as stated in the aforementioned Teter specification, it is usually necessary, when employing sodium chloride as the chloridizing agent, to subject the zinciferous material to two or even more consecutive chloridizing sintering treatments before the cadmium content is sufficiently reduced to permit the production of high grade zinc products by the heretofore customary pyrometallurgical processes of zinc recovery.

Our present invention, based on the foregoing discovery involves subjecting the zinciferous material to a heat treatment operation in the presence of a chloridizing agent and water vapor under conditions of basicity favorable to effective utilization of acidic compounds of chlorine for chloridizing cadmium and/or other contaminating metals. Such conditions of basicity are preferably brought about by avoiding the formation of strongly basic reaction products, such as sodium oxide. This may be advantageously effected by adding zinc chloride, preferably in the form of an aqueous solution thereof, to the zinciferous material, or by chloridizing a small portion of the zinc in the zinciferous material, either before the heat treatment or while it is in progress, by reagents that do not form strongly basic reaction products. Where a strongly basic reaction product is formed, the conditions of basicity characteristic of the invention may be brought about by associating with the zinciferous material (by reaction or otherwise) a suitable acidic substance or reaction product capable of neutralizing the strongly basic reaction product.

55

60

65

70

75

80

85

90

95

100

and thereby permitting effective utilization of the chloridizing agent.

The invention can be carried out in practice in a number of different ways. Merely by way of illustration, we will first describe what is now our preferred practice in treating a zinc flotation concentration containing about 65% zinc, from 3-5% lead and about 0.12% cadmium, in accordance with the principle of the invention. The concentrate is first subjected to an ordinary desulfurizing or roasting treatment carried out in any appropriate roasting apparatus. The roasting need not be carried to completion as any residual sulfide sulfur serves as fuel in the subsequent sintering operation and thus replaces an equivalent amount of coal. The roasted concentrate is then mixed with an appropriate amount of coal and a solution of zinc chloride containing the proper amount of water and of zinc chloride. If the concentrate is completely roasted, 5% by weight of anthracite dust coal or coke fines has been found to give satisfactory results. The amount of water used must be that which gives the resulting mixture the proper consistency. Proper consistency may be defined as that consistency which gives a maximum porosity consistent with sufficient strength of structure to prevent collapse when the mixture is subjected to the down-draft of a Dwight Lloyd sintering machine. In this particular example, the charge prepared for sintering contains approximately 30% by weight of water. A sufficient amount of zinc chloride should be present in the mixture to provide a slight excess of chlorine over that theoretically required to chloridize all of the cadmium and lead in the zinciferous material. Zinc chloride in large excess of that required to chloridize the cadmium and lead is harmful since it causes an objectionable loss of zinc. In the example under discussion, 5% by weight of zinc chloride gives satisfactory results.

The mixing and heat treatment operations of the invention may be advantageously carried out in a Dwight-Lloyd sintering apparatus with the mixing, crushing and screening equipment commonly employed therewith. The mixing should be so conducted as to yield a fluffy product rather than a dense, compact one. The sintering operation should be conducted to produce uniform, porous sinter in order to obtain the maximum removal of cadmium and lead. The suction in the windbox of the sintering machine is regulated to draw a sufficient amount of air through the charge so that the sintered product discharged at the end of the machine is not red hot and fuming. The volatilized fume may be collected by any appropriate method and its cadmium, lead and zinc content recovered. The lead and cadmium may be

recovered by taking the fume into aqueous solution and replacing lead and cadmium by zinc. If desired, the resulting zinc chloride solution may be returned for use in the sintering operation, supplemented by the addition of such small amount of fresh zinc chloride, or other appropriate source of chlorine including even sodium chloride, as may be necessary to compensate for losses in chlorine.

A very substantial elimination of cadmium and lead is effected by a single chloridizing sintering operation carried out in the manner just described. Thus, for example, starting with a roasted flotation concentrate containing about 65% zinc, from 3-5% lead and about 0.12% cadmium, a single chloridizing sintering treatment carried out as described produced a sintered product of substantially the same zinc content and containing less than 0.0025% cadmium and less than 0.1% lead. Under the heretofore customary procedure using sodium chloride as the chloridizing agent, as described in the aforementioned Teter application, at least two consecutive chloridizing sintering operations are necessary to effect the reduction in the cadmium and lead content of this same roasted concentrate which is effected in a single chloridizing sintering operation conducted in accordance with our invention.

The improved results attained by the practice of the invention are due to the action, as the chloridizing agent, of zinc chloride in the absence of strongly basic products. It is our belief that during the sintering operation the zinc chloride, zinc oxide and water, present in the mixture undergoing treatment, react to form zinc oxychloride. The zinc oxychloride is not stable at the temperature attained during sintering and probably dissociates into zinc oxide and hydrochloric acid. The ultimate reaction, omitting intermediate steps, may be expressed by the following equation:



The hydrochloric acid formed in this manner chloridizes cadmium and lead as well as more zinc. The cadmium chloride and lead chloride are volatilized and driven out of the charge while the zinc chloride is again converted to zinc oxide and hydrochloric acid as represented by the foregoing equation. Thus, by the practice of the invention, cadmium and lead are volatilized as chlorides without volatilizing any appreciable amount of zinc chloride, in spite of the fact that zinc chloride has a higher vapor pressure than either cadmium chloride or lead chloride.

The superior action of zinc chloride as a chloridizing agent for removing cadmium and/or lead from zinciferous material is attributable we believe to (1) its strong chemical attraction for water, (2) the fact that it is an excellent flux, and (3) the fact that it

is readily hydrolyzed and forms an oxide which is not strongly basic.

The strong chemical attraction of zinc chloride for water increases the amount of water required to attain the proper consistency of the zinciferous charge prepared for sintering. It is also significant that the use of zinc chloride not only requires the use of additional water to attain proper consistency, but that this water is not driven off, during sintering, until a higher temperature is reached. This additional water in the charge prepared for sintering has three advantages, namely:

(a) The drying out of the bed, especially the lower part, is retarded; thus maintaining the proper consistency for a longer time. This explains the fact that in practice the use of zinc chloride makes it possible to obtain a more uniform sinter.

(b) The formation of more hydrochloric acid by the hydrolysis of zinc chloride is made possible, the reaction being represented by the equation hereinbefore given.

(c) The increase in the hydrolysis of zinc chloride caused by the additional water will also decrease the loss of zinc by volatilization.

The fact that zinc chloride is an excellent flux promotes, we believe, the release of cadmium from certain ores in which it is intimately interlocked with the zinc.

In the hydrolysis of zinc chloride, represented by the foregoing equation, there results an oxide ( $ZnO$ ) which is not strongly basic and hydrochloric acid, a powerful chloridizing agent. Due to the absence of any strongly basic reaction product, the hydrochloric acid, resulting from the hydrolysis of zinc chloride, is available in large part, if not wholly, for the chloridizing of cadmium and lead. On the other hand, when using sodium chloride as the chloridizing agent, hydrochloric acid, when formed as an intermediary reaction product, is at least partially neutralized by sodium oxide (also an intermediary reaction product) which is a strong base.

The action of sodium chloride, as the chloridizing agent, may be summarized by the following equations:



Consideration of the foregoing equations shows that, in addition to the detrimental effect of the strongly basic intermediary reaction product formed, there is another very important factor to be considered, namely the speed of reaction. Using zinc chloride as a chloridizing agent, in accordance with our invention, only one reaction (zinc chloride plus water) is necessary to form hydrochloric acid—the active chloridizing agent. However, when sodium chloride is used as a chloridizing agent, the preliminary, and relative-

ly slow, reaction (1) must take place before the zinc chloride, necessary for the second reaction, can be formed, thus delaying the ultimate chloridization of cadmium and lead.

The importance of this time factor is shown, for example, in comparing two successive sinters, each using  $2\frac{1}{2}\%$  sodium chloride, with one sinter using 5% sodium chloride. The first procedure gives much better impurity elimination than the second. One reason for this is undoubtedly the fact that in the former case the time for reaction is twice as long as in the latter. The same beneficial effect of increasing the time for reaction is obtained in the practice of the present invention by increasing the speed of reaction in consequence of the elimination of the preliminary reaction (foregoing equation 1) resulting from the use of zinc chloride as the chloridizing agent.

It is undoubtedly true that in any chloridizing sintering of zinciferous material the chloridizing agent at first forms chlorides of the available metals, including zinc, cadmium and lead. The relative amount of zinc chloride is large due to the preponderance of zinc over the other metals in the zinciferous material, and the chloridization of the other metals by this first reaction is incomplete. As previously intimated, it is our belief that the remaining cadmium and lead are chloridized at the expense of the zinc chloride. Where, therefore, as in our present invention, the presence of zinc chloride and the absence of strongly basic products are assured, substantially complete elimination of the usual percentages of the contaminating metals is effected in a single chloridizing sintering operation.

The importance of water in the reactions necessary for efficient chloridization has already been pointed out. From a physical standpoint water is necessary to obtain the desired uniform porosity of the bed. During the sintering operation there is an inevitable tendency for the bottom of the bed to dry out before the operation has reached completion. This usually results in poorer sinter in the bottom part of the bed than in the top. It is evident that this effect would be decreased by increasing the amount of water in the charge.

From a chemical standpoint water is essential, because it reacts with zinc chloride to form hydrochloric acid and zinc oxide thus serving the double purpose of facilitating the chloridization of lead and cadmium, by the production of hydrochloric acid, and reducing the zinc loss by converting volatile zinc chloride into non-volatile zinc oxide. From the law of mass action it is evident that these desirable effects would be increased by increasing the amount of water in the charge.

The use of zinc chloride, as the chloridizing agent, permits the use of relatively more

water in the charge prepared for sintering, as hereinbefore explained. We have further found that relatively more water can be added to the charge, without rendering the charge too doughy or pulpy for the production of sufficient porosity during the subsequent sintering, if the mechanical work done to effect mixing be restricted to that absolutely necessary to secure a proper blending of the zinciferous material, fuel, water and reagents. In practice, the amount of work done in mixing the charge may be decreased by decreasing the time of mixing and/or by modifying the heretofore customary method of mixing the charge for sintering. Thus, decreasing the mixing time in a Werner-Pfleiderer laboratory batch mixer from 3 minutes to 1 minute permits a substantial increase in the water content of the charge. Also, by modifying a Dwight-Lloyd mixer so as to shorten the path of the mixture and by using a relatively shallow bed, the permissible water content of the charge may be increased enormously over that possible when the mixing is done in a pug mill or in the usual Dwight-Lloyd mixer. The use of the shallow bed permits a certain amount of rolling of the mixture which causes lumps to form. It has been found possible to prevent lump formation by increasing the speed of the paddles. The formation of rings of wet ore in the spaces between the paddles can be overcome either by widening the paddles or by increasing the number of paddles. The effectiveness of varying the water content of the charge by varying the work done in mixing is different for different ores. In general, it is greatest with a very fine particle size ore such as a flotation concentrate and becomes substantially negligible with coarse gravity or magnetic concentrates.

The proper amount of water to be incorporated in the charge prepared for sintering will depend on the chemical composition of the ore or other zinciferous material, on the particle size of the ore, on the mixing procedure, and on the chloridizing agent used. Treating a roasted flotation concentrate, such as hereinbefore described, the charge prepared for sintering may contain 30% by weight of water, whereas in the treatment of a relatively coarse gravity or magnetic concentrate the permissible amount of water incorporated in the charge may be as little as 5% by weight. It has been found harmful to wet the zinciferous material at any time prior to the preparation of the mixed charge for sintering. This has been found to be the case even where the material is again dried before the mixing operation.

Another factor which we have found to materially influence the efficiency of cadmium and lead elimination is the length of time of ignition in the sintering operation. In the past, it has, of course, been realized that the

ignition time must be sufficient to thoroughly ignite the top of the bed, but any extension of the time beyond this period was considered unnecessary. We have found it advantageous to prolong the ignition of the sintering charge beyond the time necessary to ignite the surface layer, the optimum time of ignition depending on the ignition apparatus employed. We have obtained a marked improvement in the elimination of cadmium and lead by extending the ignition period to a duration six times that required to ignite the top of the charge.

The elimination of the cadmium and lead, in accordance with the invention, may be accomplished by the use of chloridizing agents other than zinc chloride, but in any case zinc chloride should be formed either prior to or during the heat treatment operation. Thus, the zinc chloride may be formed by chloridizing part of the zinc in the material to be treated. This can be conveniently accomplished, especially with oxidized or roasted ores, by adding dilute hydrochloric acid to the zinciferous material in place of the aqueous solution of zinc chloride hereinbefore described. Hydrochloric acid may be formed in the zinciferous material by adding thereto sulfuric acid and sodium chloride, in which case the sulfuric acid reacts in part with the sodium chloride to form sodium sulfate and hydrochloric acid. Sodium oxide may, it is true, be subsequently formed by the thermal decomposition of the sodium sulfate during the ensuing sintering operation, but this decomposition liberates sulfur trioxide and/or sulfur dioxide at the same time, the acidity of which tends to reduce the basicity due to the formation of the sodium oxide, and to neutralize its deleterious effects. Furthermore, the sulfuric acid likewise forms zinc sulfate with the zinc oxide present in the zinciferous material. This zinc sulfate is decomposed during the subsequent sintering to zinc oxide, a base of moderate strength, and sulfur trioxide and/or sulfur dioxide, strong acids. These reactions set up conditions that inhibit the strongly basic intermediary reaction product (sodium oxide) from diminishing the effectiveness of the chloridizing agent. It is evident from these last discussed reactions that zinc sulfate may be used (as a substitute for sulfuric acid) with sodium chloride or other alkaline or alkaline earth chloride to provide the active chloridizing agent under conditions incapable of rendering the chlorine present unavailable for its contemplated useful chloridizing action.

It is to be understood that sodium chloride is mentioned in the preceding paragraph merely by way of example and that this phase of the invention is not restricted thereto. Other alkaline or alkaline earth chlorides can be used, such as calcium chloride, barium chloride, and the like. It is further to be

understood that use may be made of acids other than sulfuric acid which give substantially the same end results in the sintering operation.

While we have particularly specified a sintering operation by blast-roasting as our preferred type of heat treatment operation, it is to be understood that the invention is not restricted to that particular type of heat treatment. In its broad aspect, the invention may be carried out by any heat treatment operation adapted to effect the contemplated chloridizing action. It is characteristic of the invention that the heat treatment, in conjunction with the chloridizing agent and water vapor under conditions of basicity incapable of rendering the chlorine compounds present unavailable for the contemplated useful chloridizing action, effects the removal of the contaminating metals by volatilization. The gaseous products of the heat treatment operation should be removed under conditions substantially inhibiting condensation of any metal chlorides within the charge undergoing treatment. Such removal of the gaseous products of the operation may be advantageously accomplished by maintaining an appropriate gaseous current through the charge of zinciferous material while subjected to the heat treatment.

The purity of commercial zinc products is graded according to their cadmium, lead and iron content. The following specifications have been adopted for zinc metal (spelter) in the United States by the American Society for Testing Materials.

|                          | High grade | Intermediate | Brass special | Selected | Prime western |
|--------------------------|------------|--------------|---------------|----------|---------------|
| Cadmium, not more than   | 0.07%      | 0.50%        | 0.50%         | 0.75%    | No limit      |
| Lead, not more than----- | 0.07       | 0.20         | 0.60          | 0.80     | 1.60%         |
| Iron, not more than----- | 0.03       | 0.03         | 0.03          | 0.04     | 0.08          |

While the grades shown above are the official specifications, the commercial distinctions are high grade virgin, redistilled, brass special, and prime western. High grade virgin metal comprises that made from Franklin, N. J., ores by pyrometallurgical methods, and that made from certain other zinc ores by electrolytic processes.

Applying our present invention to the treatment of zinc ores from which heretofore only the lower grades of zinc metal could be produced by customary pyrometallurgical methods, we have been able to eliminate the cadmium and lead to such an extent that zinc metal equal in purity to high grade virgin metal may be produced therefrom in a furnace of the ordinary multiple retort type. Furthermore, zinc metal containing 99.99+ % zinc may be produced from such ores treated in accordance with the invention and subsequently smelted or reduced in the form of

coked agglomerates in a vertical retort furnace with lead elimination, in accordance with the practice described in United States Patent No. 1,712,132.

We claim:—

1. The improvement in the treatment of zinciferous material containing cadmium which comprises subjecting the material to a heat treatment operation in the presence of a chloridizing agent and water vapor and under conditions of basicity favorable to effective utilization of acidic compounds of chlorine for chloridizing cadmium and thereby effecting the removal from the material by volatilization of such an amount of cadmium without substantial loss of zinc that the so-treated material is of sufficiently low cadmium content for the pyrometallurgical production of a high grade zinc product therefrom.

2. The improvement in the treatment of zinciferous material containing cadmium which comprises subjecting the material to a heat treatment operation in the presence of a chloridizing agent and water vapor and under conditions incapable of forming strongly basic reaction products and thereby effecting the removal from the material by volatilization of such an amount of cadmium without substantial loss of zinc that the so-treated material is of sufficiently low cadmium content for the pyrometallurgical production of a high grade zinc product therefrom.

3. The improvement in the treatment of zinciferous material containing cadmium which comprises subjecting the material to a sintering operation by blast-roasting in the presence of a chloridizing agent and water vapor and under conditions of basicity favorable to effective utilization of acidic compounds of chlorine for chloridizing cadmium and thereby effecting the removal from the material by volatilization of such an amount of cadmium without substantial loss of zinc that the cadmium content of the so-treated material is sufficiently low for the production of high grade zinc products therefrom by customary pyrometallurgical methods.

4. The improvement in the treatment of zinciferous material containing cadmium which comprises subjecting the material to a sintering operation by blast-roasting in the presence of a chloridizing agent and water vapor and under conditions incapable of forming strongly basic reaction products and thereby effecting the removal from the material by volatilization of such an amount of cadmium without substantial loss of zinc that the cadmium content of the so-treated material is sufficiently low for the production of high grade zinc products therefrom by customary pyrometallurgical methods.

5. The improvement in the treatment of

zinciferous material containing cadmium which comprises subjecting the material to a sintering operation by blast-roasting in the presence of zinc chloride and water vapor and thereby effecting the removal from the material by volatilization of such an amount of cadmium without substantial loss of zinc that the cadmium content of the resulting material is sufficiently low for the production of high grade zinc products therefrom by customary pyrometallurgical methods.

6. The improvement in the treatment of zinciferous material containing cadmium which comprises mixing the material with a combustible agent and an aqueous solution of hydrochloric acid, and subjecting the resulting mixture to a sintering operation by blast-roasting in the course of which a large proportion of the initial cadmium content of the zinciferous material is removed by volatilization without substantial loss of zinc.

7. The improvement in the treatment of zinciferous material containing cadmium which comprises mixing the material with an aqueous solution of hydrochloric acid, and heating the resulting mixture in the presence of water vapor and thereby effecting the removal from the material by volatilization of an economically significant amount of cadmium without substantial loss of zinc.

8. The improvement in the treatment of zinciferous material containing cadmium which comprises mixing the material with an aqueous solution of a chloridizing agent until there is uniformly distributed throughout the material a sufficient amount of zinc chloride to chloridize all the cadmium therein, subjecting the resulting mixture to a heat treatment operation in the presence of water vapor, and maintaining a gaseous current through the mixture while subjected to said heat treatment whereby a large proportion of the initial cadmium content of the zinciferous material is removed by volatilization without substantial loss of zinc.

9. The improvement in the treatment of zinciferous material containing cadmium which comprises mixing the material with a combustible agent and with an aqueous solution of a chloridizing agent until there is uniformly distributed throughout the material a sufficient amount of zinc chloride to chloridize all the cadmium therein, and subjecting the resulting mixture to a sintering operation by blast-roasting in the course of which a large proportion of the initial cadmium content of the zinciferous material is removed by volatilization without substantial loss of zinc.

10. The improvement in the treatment of zinciferous material containing cadmium and/or lead which comprises subjecting the material to a heat treatment operation in the presence of a chloridizing agent and water vapor and under conditions of basicity favor-

able to effective utilization of acidic compounds of chlorine for chloridizing cadmium and/or lead and thereby effecting the removal from the material by volatilization of an economically significant amount of cadmium and/or lead without substantial loss of zinc.

11. The improvement in the treatment of zinciferous material containing cadmium and/or lead which comprises subjecting the material to a heat treatment operation in the presence of a chloridizing agent and water vapor and under conditions incapable of forming strongly basic reaction products and thereby effecting the removal from the material by volatilization of an economically significant amount of cadmium and/or lead without substantial loss of zinc.

12. The improvement in the treatment of zinciferous material containing cadmium and/or lead which comprises subjecting the material to a sintering operation by blast-roasting in the presence of a chloridizing agent and water vapor and under conditions of basicity favorable to effective utilization of acidic compounds of chlorine for chloridizing cadmium and/or lead and thereby effecting the removal from the material by volatilization of an economically significant amount of cadmium and/or lead without substantial loss of zinc.

13. The improvement in the treatment of zinciferous material containing cadmium and/or lead which comprises subjecting the material to a sintering operation by blast-roasting in the presence of a chloridizing agent and water vapor and under conditions incapable of forming strongly basic reaction products and thereby effecting the removal from the material by volatilization of an economically significant amount of cadmium and/or lead without substantial loss of zinc.

14. The improvement in the treatment of zinciferous material containing cadmium and/or lead which comprises subjecting the material to a heat treatment operation in the presence of zinc chloride and water vapor and under conditions of basicity favorable to effective utilization of acidic compounds of chlorine for chloridizing cadmium and/or lead and thereby effecting the removal from the material by volatilization of an economically significant amount of cadmium and/or lead without substantial loss of zinc.

15. The improvement in the treatment of zinciferous material containing cadmium and/or lead which comprises subjecting the material to a heat treatment operation in the presence of zinc chloride and water vapor and under conditions incapable of forming strongly basic reaction products and thereby effecting the removal from the material by volatilization of an economically significant amount of cadmium and/or lead without substantial loss of zinc.

16. The improvement in the treatment of zinciferous material containing cadmium and/or lead which comprises subjecting the material to a sintering operation by blast-roasting in the presence of zinc chloride and water vapor and under conditions of basicity favorable to effective utilization of acidic compounds of chlorine for chloridizing cadmium and/or lead and thereby effecting the removal from the material by volatilization of an economically significant amount of cadmium and/or lead without substantial loss of zinc. 10
17. The improvement in the treatment of zinciferous material containing cadmium and/or lead which comprises subjecting the material to a sintering operation by blast-roasting in the presence of zinc chloride and water vapor and under conditions incapable of forming strongly basic intermediary reaction products and thereby effecting the removal from the zinciferous material by volatilization of a large proportion of its initial cadmium and/or lead content without substantial loss of zinc. 20
18. The improvement in the treatment of zinciferous material containing cadmium and/or lead which comprises subjecting the material to a heat treatment operation in the presence of a chloridizing agent and water vapor and under conditions of basicity favorable to effective utilization of acidic compounds of chlorine for chloridizing cadmium and/or lead, and maintaining a gaseous current through the material while subjected to said heat treatment and thereby effecting the removal from the material by volatilization of an economically significant amount of cadmium and/or lead without substantial loss of zinc. 30
19. The improvement in the treatment of zinciferous material containing cadmium and/or lead which comprises subjecting the material to a heat treatment operation in the presence of zinc chloride and water vapor and under conditions incapable of forming strongly basic reaction products, and maintaining a gaseous current through the material while subjected to said heat treatment whereby a large proportion of the initial cadmium and/or lead content of the zinciferous material is removed by volatilization without substantial loss of zinc. 40
20. The improvement in the treatment of zinciferous material containing cadmium and/or lead which comprises mixing the material with an aqueous solution of a chloridizing agent until there is uniformly distributed throughout the material a sufficient amount of zinc chloride to chloridize all the cadmium and/or lead therein, and subjecting the resulting mixture to a heat treatment operation in the course of which a large proportion of the initial cadmium and/or lead content of the zinciferous material is removed by volatilization without substantial loss of zinc. 50
21. The improvement in the treatment of zinciferous material containing cadmium and/or lead which comprises mixing the material with an aqueous solution of a chloridizing agent until there is uniformly distributed throughout the material a sufficient amount of zinc chloride to chloridize all the cadmium and/or lead therein, and subjecting the resulting mixture to a sintering operation by blast-roasting in the course of which a large proportion of the initial cadmium and/or lead content of the zinciferous material is removed by volatilization without substantial loss of zinc. 60
22. The improvement in the treatment of zinciferous material containing cadmium and/or lead which comprises mixing the material with an aqueous solution of hydrochloric acid containing sufficient chlorine to chloridize all the cadmium and/or lead therein, and subjecting the resulting mixture to a heat treatment operation in the course of which a large proportion of the initial cadmium and/or lead content of the zinciferous material is removed by volatilization without substantial loss of zinc. 70
23. The improvement in the treatment of zinciferous material containing cadmium and/or lead which comprises mixing the material with an aqueous solution of hydrochloric acid containing sufficient chlorine to chloridize all the cadmium and/or lead therein, and subjecting the resulting mixture to a sintering operation by blast-roasting in the course of which a large proportion of the initial cadmium and/or lead content of the zinciferous material is removed by volatilization without substantial loss of zinc. 80
24. The improvement in the treatment of zinciferous material containing cadmium and/or lead which comprises mixing the material with an acid and a chloride, and subjecting the resulting mixture to a heat treatment operation under conditions of basicity favorable to effective utilization of acidic compounds of chlorine for chloridizing cadmium and/or lead and thereby effecting the removal from the zinciferous material by volatilization of an economically significant amount of cadmium and/or lead without substantial loss of zinc. 90
25. The improvement in the treatment of zinciferous material containing cadmium and/or lead which comprises mixing the material with an aqueous solution of zinc chloride, and subjecting the resulting mixture to a heat treatment operation and thereby effecting the removal from the material by volatilization of an economically significant amount of cadmium and/or lead without substantial loss of zinc. 100
26. The improvement in the treatment of zinciferous material containing cadmium and/or lead which comprises mixing the material with an aqueous solution of zinc chloride, and subjecting the resulting mixture to a heat treatment operation and thereby effecting the removal from the material by volatilization of an economically significant amount of cadmium and/or lead without substantial loss of zinc. 110
27. The improvement in the treatment of zinciferous material containing cadmium and/or lead which comprises mixing the material with an aqueous solution of zinc chloride, and subjecting the resulting mixture to a heat treatment operation and thereby effecting the removal from the material by volatilization of an economically significant amount of cadmium and/or lead without substantial loss of zinc. 120
28. The improvement in the treatment of zinciferous material containing cadmium and/or lead which comprises mixing the material with an aqueous solution of zinc chloride, and subjecting the resulting mixture to a heat treatment operation and thereby effecting the removal from the material by volatilization of an economically significant amount of cadmium and/or lead without substantial loss of zinc. 130

and/or lead which comprises mixing the material with an aqueous solution of zinc chloride, subjecting the resulting mixture to a heat treatment operation, and maintaining a 5 gaseous current through the material while subjected to said heat treatment and thereby effecting the removal from the material by volatilization of an economically significant amount of cadmium and/or lead without 10 substantial loss of zinc.

27. The improvement in the treatment of zinciferous material containing cadmium and/or lead which comprises mixing the material with an aqueous solution of zinc chloride, subjecting the resulting mixture to a 15 sintering operation by blast-roasting and thereby effecting the removal from the material by volatilization of an economically significant amount of cadmium and/or lead 20 without substantial loss of zinc.

28. The improvement in the treatment of zinciferous material containing cadmium and/or lead which comprises mixing the material with an aqueous solution of zinc chloride, subjecting the resulting mixture to a 25 heat treatment operation and thereby effecting the removal from the material by volatilization of an economically significant amount of cadmium and/or lead without 30 substantial loss of zinc, forming an aqueous solution of the volatilized chlorides and replacing cadmium and/or lead therein by zinc, and utilizing the resulting aqueous solution of zinc chloride for mixture with additional zinciferous material.

29. The improvement in the treatment of zinciferous material containing cadmium and/or lead which comprises mixing the material with an aqueous solution of zinc chloride, subjecting the resulting mixture to a 40 sintering operation by blast-roasting and thereby effecting the removal from the material by volatilization of an economically significant amount of cadmium and/or lead 45 without substantial loss of zinc, forming an aqueous solution of the volatilized chlorides and replacing cadmium and/or lead therein by zinc, and utilizing the resulting aqueous solution of zinc chloride for mixture with 50 additional zinciferous material.

30. The improvement in the treatment of zinciferous material containing cadmium and/or lead which comprises mixing the material with sulphuric acid and a chloride, and 55 subjecting the resulting mixture to a heat treatment operation and thereby effecting the removal from the zinciferous material by volatilization of an economically significant amount of cadmium and/or lead without 60 substantial loss of zinc.

31. The improvement in the treatment of zinciferous material containing cadmium and/or lead which comprises mixing the material with zinc sulfate and a chloride, and 65 subjecting the resulting mixture to a heat

treatment operation and thereby effecting the removal from the zinciferous material by volatilization of an economically significant amount of cadmium and/or lead without substantial loss of zinc.

32. The improvement in the treatment of zinciferous material containing cadmium and/or lead which comprises incorporating a substantial amount of water within the mass of the material with the minimum amount 75 of work to form a fluffy mixture, and subjecting the resulting fluffy mixture to a sintering operation by blast-roasting in the presence of zinc chloride and thereby effecting the removal from the material by volatilization of an economically significant amount of cadmium and/or lead without substantial loss of zinc.

33. The improvement in the treatment of zinciferous material containing cadmium and/or lead in which the material is subjected to a sintering operation by blast-roasting in the presence of a chloridizing agent and water vapor characterized by subjecting the charge prepared for sintering to an ignition period prolonged several times beyond the time required to ignite the surface of the charge.

In testimony whereof we affix our signatures.

HOWARD M. CYR.  
ROBERT K. WARING.

95

100

105

110

115

120

125

130